

E. C. SPRAGUE & A. M. WILLIAMSON,  
METHOD OF TREATING CARBON ARTICLES OF LOW INITIAL CONDUCTIVITY,  
APPLICATION FILED MAR. 20, 1912.

1,030,620.

Patented June 25, 1912.

2 SHEETS-SHEET 1.

Fig. 1.



Fig. 2.



Witnesses:

Robert C. Sulziger

C. H. Potter

Inventors:

Edward C. Sprague,  
Arthur M. Williamson,

By Edward C. Sprague, Arthur M. Williamson  
Met 45

E. C. SPRAGUE & A. M. WILLIAMSON.  
METHOD OF TREATING CARBON ARTICLES OF LOW INITIAL CONDUCTIVITY.  
APPLICATION FILED MAR. 20, 1912.

1,030,620.

Patented June 25, 1912.

2 SHEETS-SHEET 2.

Fig. 5.



Fig. 4.



Fig. 5.



Witnesses:

Robert J. Hulsiizer.

C. H. Potter.

Inventors:

Edmund C. Sprague,  
Arthur M. Williamson,  
by Byers, Townsend & Brillenstein,  
Attys.

# UNITED STATES PATENT OFFICE.

EDMUND C. SPRAGUE AND ARTHUR M. WILLIAMSON, OF NIAGARA FALLS, NEW YORK,  
ASSIGNORS TO INTERNATIONAL ACESON GRAPHITE COMPANY, OF NIAGARA  
FALLS, NEW YORK, A CORPORATION OF NEW JERSEY.

## METHOD OF TREATING CARBON ARTICLES OF LOW INITIAL CONDUCTIVITY.

1,030,620.

Specification of Letters Patent. Patented June 25, 1912.

Application filed March 20, 1912. Serial No. 684,990.

To all whom it may concern:

Be it known that we, EDMUND C. SPRAGUE and ARTHUR M. WILLIAMSON, citizens of the United States, residing at Niagara Falls, 5 in the county of Niagara and State of New York, have invented certain new and useful Improvements in Methods of Treating Carbon Articles of Low Initial Conductivity, of which the following is a specification.

10 This invention relates to the treatment of carbon articles, and especially to the treatment of unbaked or green carbon electrodes or the like, for the purpose of increasing their electrical conductivity.

15 The invention is applicable for the production of several classes of finished articles, depending upon the duration and other conditions of heating, and upon the character of the initial material; that is to say 20 the carbon articles may be baked or polymerized to any desired degree, or they may be graphitized.

According to the preferred embodiment 25 of the invention, green or unbaked carbon articles, of which the initial electrical conductivity is too low to permit them to be heated in a commercially practicable manner by the passage of an electric current through their mass, are charged or arranged 30 in an electric furnace in the form of piles or stacks which are preferably disposed transversely to the current path, the several piles separated from each other in the direction of current flow by a subdivided or granular resistance material. The 35 articles are initially heated by means of two or more resistance bodies laterally disposed with reference to the piles, and extending between the heads or terminals of the

40 furnace. Thereafter, when the conductivity of the carbon articles has increased sufficiently to permit such effect, a part of the current flows through the piles of articles and through the interposed resistance material, resulting in a further heating of the 45 articles by heat developed in such interposed material. By proceeding in this manner, several important advantages are secured, as hereinafter pointed out.

50 For a full understanding of the invention reference is made to the accompanying drawings, diagrammatic in character, wherein—

Figure 1 is a transverse vertical section

of an electric furnace charged with carbon articles to be treated in accordance with our invention; Fig. 2 is a longitudinal vertical section thereof, the central portion being broken away; Fig. 3 is a diagrammatic representation of the temperature variations in certain portions of the furnace during an illustrative furnace run; Fig. 4 is a horizontal section of one end of a furnace provided with means for separately controlling the temperature of the heating cores; and Fig. 5 is a transverse vertical section of a furnace having three heating cores.

In said drawings, 1, 1 indicates articles of carbon, as for example green carbon electrodes which are to be baked or graphitized. Said articles are shown as disposed in a series of piles 2, arranged transversely with respect to the longest dimension of the furnace and to the path of the current between the terminal heads or electrodes 3, 4. The several articles 1, constituting a single pile 2, are superposed in contact with each other or very slightly separated, it being preferred to prevent such actual contact as might result in welding the articles together by the use of thin layers or films of fine carbon or carbon dust. The several piles 2 are separated from each other by layers 5 of granular conductive carbon, for which purpose coke, which has undergone heating in a previous furnace operation and has been thereby rendered conductive, is well suited. The end piles of the series are maintained in conductive relation with the inner ends of the electrodes 3, 4 by granular layers of like material designated by the reference numeral 6.

7, 7 represent longitudinal cores of granular or subdivided conductive material, preferably of the same character as that constituting the intermediate layers 5. These cores are properly proportioned with reference to the current to be employed, to carry the greater portion or all of the current during the earlier stages of the heating operation. 8 represents an insulating mixture, as for example a mixture of coke and sand, which completely embeds or surrounds the articles to be heated or converted, being preferably prevented from direct contact therewith above and below the piles by carbon beds 7<sup>a</sup>, 7<sup>a</sup> of materially lower conduc-

tivity than the heating cores 7. This lower conductivity may be assured for instance either by using for the layers 7<sup>a</sup> a carbon having a higher specific resistance than that of the heating cores, or by using carbon like that of the heating cores but in a comparatively loose state of aggregation. The principal purpose of the layers 7<sup>a</sup> is to protect the carbon articles from the silica of the bedding mixture 8. This bedding mixture 8 may be in lateral contact with the heating cores 7, 7. The entire charge, including the embedding material, is usually inclosed by removable retaining walls 9, carried by a permanent base or furnace-bed 10, which also carries the permanent head walls 11. The result of disposing such longitudinal cores in the described relation to the piles of carbon articles, is that these piles, and the articles constituting them, are initially heated chiefly from their ends, the term "ends" being applied to those portions of the piles which are adjacent the cores, irrespective of the form or dimensions of the individual piles or of the articles composing them. Under these conditions, the ends of the piles are brought to a temperature above that of the intermediate portions, and the mode of heating is such that there occurs, as nearly as may be practicable, a regular rise in the temperature of all portions of the articles, the higher temperature of the end portions being however maintained for a considerable proportion of the run and preferably to or nearly to the conclusion of the heating stage. This preferred condition will be apparent from an inspection of the temperature curves (Fig. 3) of an illustrative furnace run, having for its purpose the baking of green carbon electrodes. The curves show the general course of the temperature, neglecting minor variations. The several curves were plotted from the readings of pyrometers A, B, C, D, E located at points as indicated in Fig. 1, C being in the vertical axial plane of the furnace; B and D at points equally spaced on opposite sides of this plane, and A and E in the heating cores adjacent the ends of the piles. It will be noted, in this particular example, that the ends of the piles, that is to say the portions thereof adjacent the longitudinal cores, are maintained at a temperature ranging materially above the interior portions throughout the greater part of the heating stage. During the cooling stage, the conditions are reversed, owing to the more rapid loss of heat from the ends of the piles, although this effect is minimized by the heat-insulating packing. All portions of the articles may attain their maximum temperature at approximately the same time, and, under ideal conditions, this maximum temperature should be approximately the same for all portions of the articles. When such condi-

tions are even measurably attained, it is found that the results are excellent, both as regards economy of current and of time, and the condition of the product with respect to uniformity, freedom from cracks or other defects, etc.

The longitudinal cores should be as nearly as practicable of the same cross-section and conductivity, in order that the piles may be equally heated from their opposite ends; however, it may occur in practice that there will be some variation in this respect and when such variation exists, the core which shows the higher initial conductivity will tend to increase in conductivity at a higher rate, thereby increasing an initially slight difference to an extent which may lead to material irregularities. According to the present invention, this tendency is obviated by providing means for independently controlling the current in the cores. This is very simply effected by providing independent electrical connections to the cores, at least at one end thereof. This may be done, for example, as illustrated in Fig. 4, by vertically subdividing one or both of the furnace heads or terminal electrodes, for example by a vertical body of concrete or other refractory insulating material indicated at 12, thus subdividing the furnace head 4 into two portions 13, 14, each having its own system of bus-bars 15, 16. With this provision, the temperature of either core may be controlled, either by interposing a resistance in the circuit leading to one of the cores, or, and usually more simply, by merely interrupting the current through the core having the higher temperature, until the temperature of the cores have become approximately the same. This procedure may be repeated one or more times, as conditions may require, and is particularly useful in the earlier stages of the heating. In case further polymerization of the articles or their graphitization is desired, the maximum temperature and the duration of the heating will be properly increased, as will be readily understood by those skilled in this art; but in order to secure the best results, in such cases, also, the ends of the piles should be maintained during the greater part at least of the heating stage at a temperature above that of the central portions, and all portions of the piles should attain their maxima at approximately the same time, such maxima being, within reasonable and practicable limits, the same for all portions of the piles.

Our invention is not restricted to the maintenance of the particular temperature relations above-described, inasmuch as the conditions of heating should be adapted to the form and dimensions of the articles heated, in order to secure the most favorable results in any particular case. As a

rule, where the form of the articles permits such course, the piles are so disposed that their longest dimension is transverse to the path of the current between the heads or terminals; and in most cases the individual articles constituting the piles are disposed in like manner. Obviously, however, the precise arrangement adopted as most advantageous will depend upon the size and form of the articles to be treated. In certain cases, it may be desirable to provide three or more parallel heating cores, as shown in Fig. 5, means being preferably provided, as above described, for the separate temperature control of the cores.

It will be observed that under the conditions herein described, the initial heating is principally or chiefly from the opposite ends of the piles, until the articles comprising the piles have attained a considerable degree of electrical conductivity; and that thereafter an increasing proportion of the current is transmitted through the articles and through the interposed resistance layers so that the piles are heated throughout their length, by which is meant that dimension which is transverse with respect to the cores and the current path, the heating from the ends being, however, continued to the degree necessary to secure, within reasonable limits, an ultimate uniformity of treatment.

We claim:

1. The method of treating carbon articles of low initial conductivity in an electric resistance furnace, which consists in disposing said articles between the electrodes in a series of piles with interposed resistance material, and electrically heating said piles chiefly from the opposite ends thereof until the articles are rendered electrically conductive.

2. The method of treating carbon articles of low initial conductivity in an electric resistance furnace, which consists in disposing said articles between the electrodes in a series of piles with interposed resistance material, electrically heating said piles chiefly from the opposite ends thereof until the articles are rendered electrically conductive, and thereafter heating said piles throughout their length by heat developed in said interposed resistance material.

3. The method of treating carbon articles of low initial conductivity in an electric resistance furnace, which consists in disposing said articles between the electrodes in a series of piles with interposed resistance material, electrically heating said piles chiefly from the opposite ends thereof, until the articles are rendered electrically conductive, thereafter heating said piles throughout their length by heat developed in said interposed resistance material, and maintaining throughout the greater part of the heating stage a higher temperature in the

ends of the piles than in the interior portions thereof.

4. The method of treating carbon articles of low initial conductivity in an electric resistance furnace, which consists in disposing said articles between the electrodes in a series of piles with interposed resistance material, electrically heating said piles chiefly from the opposite ends thereof, until the articles are rendered electrically conductive, thereafter heating said piles throughout their length by heat developed in said interposed resistance material, maintaining throughout the greater part of the heating stage a higher temperature in the ends of the piles than in the interior portions thereof, and finally bringing all portions of said piles to approximately the same maximum temperature.

5. The method of treating carbon articles of low initial conductivity in an electric resistance furnace, which consists in disposing said articles between the electrodes in a series of piles with interposed resistance material, electrically heating said piles chiefly from the opposite ends thereof, until the articles are rendered electrically conductive, thereafter heating said piles throughout their length by heat developed in said interposed resistance material, maintaining throughout the greater part of the heating stage a higher temperature in the ends of the piles than in the interior portions thereof, and finally bringing all portions of said piles at approximately the same time to approximately the same maximum temperature.

6. The method of treating carbon articles of low initial conductivity in an electric resistance furnace, which consists in initially heating said articles chiefly from their opposite ends until they are rendered electrically conductive, and thereafter heating them with substantial uniformity throughout their length.

7. The method of treating carbon articles of low initial conductivity in an electric resistance furnace, which consists in disposing said articles in a series of piles with interposed resistance material, electrically heating said piles chiefly from the opposite ends thereof until the articles are rendered electrically conductive, and independently controlling the application of heat to the respective ends of said piles.

8. The method of treating carbon articles of low initial conductivity in an electric resistance furnace, which consists in disposing said articles in a series of piles with interposed resistance material, said piles arranged transverse to the current path, electrically heating said piles chiefly from the opposite ends thereof until the articles are rendered electrically conductive, and independently controlling the application of heat to the respective ends of said piles.

9. The method of treating carbon articles of low initial conductivity in an electric resistance furnace, which consists in disposing said articles in a series of piles with interposed resistance material, electrically heating said piles chiefly from the opposite ends thereof until the articles are rendered electrically conductive, thereafter heating said piles throughout their length by heat developed in said interposed resistance material, and independently controlling the application of heat to the respective ends of said piles.

10. The method of treating carbon articles of low initial conductivity in an electric resistance furnace, which consists in disposing said articles in a series of piles with interposed resistance material, said piles arranged transverse to the current path, electrically heating said piles chiefly from the opposite ends thereof until the articles are rendered electrically conductive, thereafter heating

said piles throughout their length by heat developed in said interposed resistance material, and independently controlling the application of heat to the respective ends of said piles.

11. The method of treating carbon articles of low initial conductivity in an electric resistance furnace, which consists in initially heating said articles chiefly from their opposite ends until they are rendered electrically conductive, thereafter heating them with substantial uniformity throughout their length, and independently controlling the application of heat to the respective ends of the articles.

In testimony whereof, we affix our signatures in presence of two witnesses.

EDMUND C. SPRAGUE.

ARTHUR M. WILLIAMSON.

Witnesses:

ALBERT S. KNIGHT,

EBEN C. SPEIDEN.